

## UNITED STATES PATENT OFFICE.

ALADAR PACZ, OF CLEVELAND, OHIO, ASSIGNOR TO GENERAL ELECTRIC COMPANY,  
A CORPORATION OF NEW YORK.

## METAL AND ITS MANUFACTURE

No Drawing. Original application filed February 20, 1917, Serial No. 149,915. Divided and this  
application filed February 15, 1922. Serial No. 536,815.*To all whom it may concern:*

Be it known that I, ALADAR PACZ, a citizen of the United States, residing at Cleveland, in the county of Cuyahoga, State of Ohio, have invented certain new and useful Improvements in Metals and Their Manufacture, of which the following is a specification.

This case is a division of my application Serial No. 149,915, filed February 20, 1917.

The object of my invention is to produce tungsten metal which will retain to a much higher degree than heretofore its original properties after being subjected to high temperatures. In the case of incandescent lamp filaments, the high temperatures at which they are run have caused them to elongate and sag between their supports. This is especially noticeable in coiled filaments, and in gas filled lamps this tends to reduce the efficiency of the lamp on account of the increased cooling effect on the filament. By means of my invention the sagging is substantially eliminated and "offset" setting of the filament is substantially prevented, during a normal or commercially useful life of the lamp.

In the preferred form of my invention I bring into intimate association with tungsten a material which will have the desired influence upon the grain growth of the metal. I precipitate, simultaneously, compounds from which the metal is to be directly reduced with the material or compound which is to accomplish the desired result. The material after precipitation will remain in intimate association with the metal even after the same has been reduced by the ordinary means, i. e., reducing gases. During the subsequent formation of the metal into ingots or bars, the material should be such that it will be removed as by volatilization. A material should be used which will have a fairly high volatilization point which is preferably somewhat lower than the sintering point of the metal.

Considering my invention from the physical standpoint, the presence of the material has an influence on the grain growth of the metal. When the metal reaches the temperature at which extensive grain growth would ordinarily take place, the presence of this material intimately associated with the tungsten particles has a

marked effect on the shape and size of the tungsten grains. The ingot of tungsten thus produced, whether it be due to the fact that the grains have not reached the equilibrium grain size or to other causes, is particularly susceptible to grain growth during subsequent heat treatments.

The probable reason why filaments made according to my invention do not sag, is that the structure is comparatively coarse grained. The coarse grained filament produced by means of my invention does not "offset" so as to cut short the life of the lamp appreciably.

As hereinbefore stated, the material which is intimately incorporated with the metal should be such that it will be volatilized out after the metal has reached the temperature of rapid grain growth. Tungsten above 1500° C. shows rapid grain growth, and I may use silica, or compounds containing it, as the material, incorporated very intimately as heretofore explained. By the time the tungsten has reached the sintering temperature the silica and the compounds containing it are volatilized out.

In order to comply fully with the requirements of the patent statutes, I will now describe one method or process embodying my invention and also modifications thereof. However, it is to be understood that the scope of my invention is such that many changes and substitutions will readily suggest themselves to those skilled in the art, and, as indicated, in the appended claims, are to be considered as forming part thereof.

A fusion of materials is first made which is quite similar to that disclosed in my Patent Number 1,299,017 issued April 1, 1919. 1400 grams of commercial tungstic acid, 620 grams commercial sodium carbonate, 620 grams commercial potassium carbonate, and 300 grams commercial sodium nitrate are mixed with water to a paste. I have found that half or more of the potassium carbonate may be replaced by sodium carbonate without affecting the results, the object being to obtain a good fusion. This paste is dried on a hot plate and fused with a torch for about fifteen minutes, after which the fusion is dissolved in water, filtered and diluted to about six liters. This we will term solution A.

A mixture is then made of 180 grams com-

mercial silicic acid, 620 grams commercial  $K_2CO_3$  and 150 grams commercial  $NaNO_3$  with water to a paste which is dried and fused. The object is to produce a silicate 5 which will be readily incorporated with the tungstic acid in the subsequent portion of the process. An alkaline silicate such as produced by the specific example given is readily soluble and efficacious for this purpose. The fusion is dissolved in water, filtered and diluted to 5 liters. This may be termed solution B.

About 250 cubic centimeters of solution B is added to 3 liters of solution A. The 15 whole solution is then boiled with steam and poured into a boiling solution containing about 1500 cubic centimeters of HCl and 1500 cubic centimeters of  $H_2O$ , preferably through a funnel. The precipitate is 20 allowed to settle, the liquid decanted, and the precipitate separated by filtration. The precipitate is then washed with hot  $H_2O$  until the filtrate becomes milky. The 25 precipitate is then dried and ignited in a quartz dish. It is reduced in hydrogen in boats, each boat containing about 100 grams. The metal thus produced may be termed metal A.

The metal A may be pressed up and sintered to produce tungsten slugs which may 30 be drawn into filaments having the non-sag and other characteristics hereinbefore described. I prefer, however, in order to obtain greater uniformity of product to continue the operation as follows:

About 1200 grams of metal A are mixed 35 with about 1200 grams of the oxide from which metal A was reduced, the mixing being very intimate and being performed 40 preferably in a tumbling mill. The mixture is then reduced as before although 150 gram charges may be here used. The metal thus produced may be termed metal B. It 45 is then sieved, pressed into ingots, sintered and formed in the usual way as set forth in the Coolidge Patent 1,082,933.

As a modification of the above described 50 process, solution B may be added directly to the fusion from which solution A is made. This is preferably done by utilizing the proper proportion as heretofore stated of 55 solution B in making the paste which is dried and fused and dissolved to form solution A.

Another modification would be to utilize 60 combinations of  $WO_3$  and oxides of tantalum, for example  $Ta_2O_5$  or of niobium, for example  $Nb_2O_5$ , or, as before indicated, of these oxides of tantalum or niobium per se. For this purpose, instead of sodium potassium 65 silicates, potassium tantalates or niobates may be added to the solution of tungstates. (Sol. A.)

The metal obtained from the first method 70 above described I have called "218", a purely

arbitrary name. I have produced a metal differing in appearance and physical characteristics from "218" metal by adding a solution of boric acid to chemically pure  $WO_3$ , evaporizing, drying, igniting and reducing. The metal thus produced when made into wire is not superior to 218 in non-sagging or non-offsetting characteristics, but a combination of this method with that for producing "218" in which the  $WO_3$  from the latter is mixed with that from the former produces a metal which I term "Z" and which is efficacious in the production of non-sagging and non-offsetting filaments. To 75 produce this metal one method which I have practiced is to mix 1 kilogram of the tungstic oxide from which metal A is reduced in the "218" process with a solution of 12.5 grams fused  $B_2O_3$  in 500 cubic centimeters of water. This mixture is evaporated, dried, ignited and reduced. The resulting metal is blacker than "218", flows more readily and possesses at least one-third larger volume than "218" although reduced under exactly the same conditions.

The tungsten ingots produced according to my invention have usually fine grains, as for example, between 2500 and 6500 grains per square millimeter. In the case of the "218" ingots analyses have shown that the percentage of non-metallic material is below two-tenths of one per cent and in many cases below one-tenth and even one-twentieth of one per cent.

When the tungsten metal produced by any of the methods above described is made into a filamentary body, the method described in the Coolidge Patent No. 1,082,933 for drawing or otherwise working down the ingots is practiced. Where the wire is to be used at high temperatures such as in incandescent electric lamps it should be given a preliminary heat treatment or aging. This helps to secure the non-sag characteristics of the wire made according to my invention. One procedure followed with good results with the ordinary 110-115 volt lamps was to run at 30 volts for 2 minutes and then at steps of 5 volts each for two minutes, up to 60 volts. After this the wire was run at 115% voltage for 15 minutes.

The tests show that substantially all of the sagging occurs during the aging of the lamp.

What I claim as new and desire to secure by Letters Patent of the United States, is,—

1. The method of producing substantially non-sagging and non-offsetting tungsten filaments which includes producing an intimate mixture of finely divided tungsten and a compound or compounds containing oxide of tantalum or niobium or both and thereafter sintering a compacted body of said mixture.

2. The method of producing substantially non-sagging and non-offsetting tungsten filaments which includes producing an intimate mixture of finely divided tungsten and a compound or compounds containing oxide of tantalum or niobium or both, sintering a compacted body of said mixture to form an ingot and thereafter working the said ingot to filamentary form.
- 5 3. The method of producing substantially non-sagging and non-offsetting tungsten fila-
- ments which includes the incorporation with finely divided tungsten of an oxide of tantalum or niobium or both derived from potassium tantalate or niobate or both, sintering a compacted body of said mixture to form an ingot and thereafter working the said ingot to filamentary form.
- 10 15 In witness whereof, I have hereunto set my hand this 14th day of February, 1922.

ALADAR PACZ.